

# United States Patent Office

3,021,183

Patented Feb. 13, 1962

1

3,021,183

TEXTILE MATERIALS RESISTANT TO FADING  
Anthony Bernard Conciatori, Chatham, N.J., assignor to  
Celanese Corporation of America, New York, N.Y.,  
a corporation of Delaware  
No Drawing. Filed Jan. 24, 1958, Ser. No. 710,870  
15 Claims. (Cl. 8—61)

This application is a continuation-in-part of my co-pending application Serial Number 534,396, filed September 14, 1955, now abandoned.

This invention relates to dyed materials and relates more particularly to dyed organic derivative of cellulose textile materials.

The art is well acquainted with the problem of the gas-fading, which is also called acid-fading, of dyed textile material having a basis of an organic derivative of cellulose. Such gas-fading may cause a material colored with a blue anthraquinone dye to take on a reddish hue, for example. It is generally accepted that this type of fading results from the presence in the atmosphere of certain oxides of nitrogen, which oxides are produced during combustion of coal, gas or other fuels. To combat this type of fading, inhibitors comprising basic nitrogen compounds, e.g. amines, are often incorporated into the textile material, before, during, or after the dyeing thereof.

On exposure to elevated temperatures the amine-type inhibitors show a tendency to discolor the textile material. This discoloration is particularly noticeable where the textile material to which the inhibitor is applied has a basis of a cellulose ester of low hydroxyl content, since such textile materials are generally exposed during processing to much higher temperatures than are employed for textile materials made from other cellulose derivatives. For example, textile materials of cellulose acetate of low hydroxyl content, commonly known as cellulose triacetate, are usually subjected to a heat-treating operation during which the fabric temperature may reach 250° C. Also heat-treated cellulose triacetate textile materials have very high safe ironing points, on the order of 240° C. or higher, and they are therefore ironed at temperatures which are much higher than those which could be employed in the case of ordinary cellulose acetate. Both the heat-treating operation and the high temperature result in some discoloration of the textile material when an amine-type gas-fading inhibitor is present. Thus, although the discoloration caused by heat-treating may be removed by the application of bleaching agents to the material, it tends to return when the material is subsequently pressed with a hot iron.

When the amine-type gas-fading inhibitors are omitted, or when there are employed selected inhibitors of this type which exhibit a greatly decreased tendency to discolor on heating, I have observed another type of fading of the anthraquinone dyes on the textile material, even when the material is not exposed to atmospheric oxides of nitrogen to any substantial extent. This type of fading called "O-fading," I believe to be due to oxidative substances present in the atmosphere which react with the dye in the material. It is observed even on organic derivative of cellulose textile materials colored with those dyestuffs which normally have very high resistance to gas-fading, such as the blue dyestuff, 1,8-dihydroxy-4-p-(beta-hydroxyethyl)anilido-5-nitroanthraquinone. In the case of the cellulose esters of low hydroxyl content, the O-fading of the colored material is particularly noticeable where the colored material is exposed to an atmosphere containing the aforesaid oxidative substances before the colored material has been heat-treated. This may take place when a fabric is dyed and then stored before heat-treating.

2

Although O-fading is prevented to a large extent by the incorporation of the usual amine-type gas-fading inhibitors in the textile material, these inhibitors, as pointed out above, cause undesired discoloration on heating. Other disadvantages of the amine-type inhibitors are that they generally tend to decrease the light-fastness of the dyed material and increase the tendency of dyed material to pick up chlorine when the material is washed in an aqueous medium containing the usual bleaching agent comprising sodium hypochlorite. Also, they usually make the material more receptive to acid dye, thus making it difficult to obtain cross-dyed effects in fabrics comprising the organic derivative of cellulose and an animal fiber such as wool.

It is therefore an object of this invention to provide a novel textile material, having a basis of an organic derivative of cellulose which material is free from the foregoing and other disadvantages.

Another object of this invention is the provision of an organic derivative of cellulose textile material which, when dyed with anthraquinone dyes, is resistant to O-fading and will not discolor a textile.

It is a further object of this invention to provide a textile material of cellulose triacetate having incorporated therein a wash-fast inhibitor of O-fading.

Other objects of this invention will be apparent from the following detailed description and claims. In this description and claims all proportions are by weight unless otherwise indicated.

In accordance with one aspect of this invention it has been found that O-fading is inhibited by the presence in the organic derivative of cellulose textile material of aliphatic carbon-to-carbon unsaturation of a non-conjugated nature, i.e. isolated ethylenic or acetylenic bonds.

This invention finds its greatest utility when the organic derivative of cellulose is a cellulose ester of low hydroxyl content, since, as pointed out above, in the normal treatment and use of such cellulose esters the elevated temperatures employed will generally tend to discolor the usual basic nitrogenous gas fading inhibitors. These cellulose esters contain not above 0.29, preferably 0 to 0.12, hydroxyl groups per anhydroglucose unit in the cellulose molecules thereof. The invention is also applicable, however, to organic derivatives of cellulose having a higher hydroxyl content, e.g. ripened, secondary or partially esterified cellulose.

The carbon-to-carbon unsaturation may be present in the organic derivative of cellulose molecule which comprises the textile material by being bound to the anhydroglucose units through their oxygen atoms, e.g. a cellulose acetate crotonate yarn having a low free hydroxyl content and a few percent of crotonyl groups can be heat treated and dyed with normally O-fading susceptible dyes without change in color. Preferably, however, the carbon-to-carbon unsaturation is present in a substance which is added to the organic derivative of cellulose in any suitable manner before, during or after the dyeing thereof. Advantageously it is incorporated into the organic derivative of cellulose before the latter is formed into filaments. To this end the inhibitor may be added to the spinning dope, e.g. to a solution of cellulose triacetate in a methylene chloride-containing solvent, for example, a solvent comprising methylene chloride alone or admixed with a lower alkanol such as methanol, ethanol, propanol, isopropanol, or butanol or mixtures of such alkanols. However, the inhibitor may also be applied, in the form of a solution or an aqueous dispersion thereof, to the organic derivative of cellulose after it has been formed into filaments, especially where the inhibitor would be only slightly soluble in the spinning dope, e.g. dimethylallylidene pentaerythritol which has limited solubility in methylene chloride.

To produce a satisfactory degree of O-fading inhibition there should be present at least one unsaturation per 50 anhydroglucose units and preferably at least one per 30 anhydroglucose units of the organic derivative of cellulose. As noted previously, this level of unsaturation can be achieved by using as the filamentary material a cellulose derivative which is inherently an inhibitor of O-fading due to the presence of unsaturations, i.e. a cellulose derivative wherein some of the cellulose hydroxyl groups are esterified or etherified with unsaturated acids or alcohols, e.g. cellulose methallylsuccinate, allyl ether of cellulose acetate, methallyl ether of cellulose acetate propionate, and the like.

Advantageously, however, the O-fading inhibition is achieved by adding unsaturated substances to a cellulose ester of a lower alkanoic acid. Representative unsaturated additives which can be used in accordance with the present invention include diallyl phthalate, dially succinate, acrylic or crotonic acid esters of mono- or polyhydric alcohols or unsaturated polyesters of polyhydric alcohols and polycarboxylic acids. Examples of such unsaturated polyesters are the linear esters of such saturated glycols as ethylene glycol, 1,2-propylene glycol, trimethylene glycol, 1,4-butene diol, isobutylene glycol or tetramethylene glycol with such unsaturated acids as allyl succinic acid, methallyl succinic acid and itaconic acid. The unsaturated polyesters may also be formed from unsaturated glycols such as 1-allyloxy-2,3-propanediol, butenediol and butyne diol and a polycarboxylic acid which may be unsaturated, e.g. the polyester of butyne diol and methallyl succinic anhydride, or saturated, e.g. the polyester of butyne diol and succinic anhydride.

Other types of unsaturated organic compounds may also be employed. For example, a highly crotonated cellulose acetate crotonate can be added to cellulose acetate to bring the average degree of unsaturation within the recited ranges. Allyl cellulose and other ethers or esters with a high degree of unsaturation can be similarly employed. There may also be used unsaturated hydrocarbons which are compatible with the organic derivative of cellulose in the amounts present. Examples of such hydrocarbons are the liquid homopolymers of butadiene and the liquid copolymers of butadiene and styrene (e.g. the product known as "C-oil"). Unsaturated ethers and acetals can also be employed, e.g. di-acrolein acetal of pentaerythritol (dicrotonylidene pentaerythritol), triallyl cyanurate, and the like. While triallyl cyanurate contains nitrogen atoms, the compound is not basic since the nitrogen of the triazine ring is not basic and does not result in the color change occasioned by conventional basic nitrogenous gas-fading inhibitors. Those additives are preferred which have relatively high molecular weights, e.g. at least 100 and preferably above 500. Such compounds have greater fastness to washing and will not be lost through vaporization during heat-treating. The unsaturation of the inhibiting group should be non-conjugated, i.e. isolated, and is preferably in a short pendant branch rather than in the main chain of the inhibiting compound, since superior O-fading is thereby achieved. While polyesters having higher acid numbers give better O-fading resistance, they render processing somewhat more difficult so that additives of lower acid numbers are preferred.

The preferred additives are non-volatile linear polyesters of molecular weights of at least about 500, possessing non-conjugated unsaturations in short side chains, and having acid numbers below about 50.

The proportion of unsaturated additive employed is desirably in the range of about 1 to 10% by weight of the cellulose derivative, preferably about 1 to 3%. Advantageously, there should not be used an amount of the inhibitor larger than that which is compatible with the organic derivative of cellulose or an amount sufficient to change appreciably the physical properties of said organic derivative of cellulose.

As noted previously, best results are obtained when the ester to which the inhibitor is added is a cellulose acetate of very high acetyl value, preferably of acetyl value 61 to 62.5%, calculated as combined acetic acid. 5 However, other organic acid esters of low hydroxyl content may be employed. Examples of such other esters are cellulose propionate, cellulose butyrate, cellulose acetate-propionate, cellulose acetate-butyrate and cellulose acetate-formate. It is to be understood, of course, that 10 the unsaturated O-fading inhibitors may also be incorporated into textile materials having a basis of other organic derivatives of cellulose such as those cellulose esters of higher hydroxyl content, e.g. cellulose acetate of acetyl value 53 to 56%, calculated as combined acetic acid.

15 The coloring of the textile material may be carried out in a manner well known to the art, preferably by applying one or more dyestuffs of the type known as dispersed cellulose acetate dyestuffs. Thus, the material may be immersed in a heated aqueous bath having a temperature of, for example, 60 to 95° C. and containing one or more dispersed cellulose acetate dyestuffs together with a dispersing agent therefor, such as sodium lignosulfonate, sulfonated naphthalene-formaldehyde condensation product or soap. Practically any desired hue may be imparted to 20 the material by the use of appropriate mixtures of dyestuffs, as by using mixtures of varying amounts of red, blue and yellow dyestuffs.

25 Preferably the blue dyestuff used is of the type which is highly resistant to gas-fading. This type of dyestuff 30 may be described as those which show negligible fading when applied in the amount of 0.3% based on the fabric weight and in the absence of a gas-fading inhibitor to a textile fabric of cellulose acetate of acetyl value 61.5%, and subjected to 3 units of gas-fading exposure 35 in accordance with Test Method 23-52 as given in the Technical Manual and Yearbook of the American Association of Textile Chemists and Colorists 1954, page 87. Specific examples of such dyestuffs are 1,8-dihydroxy-40 p - (beta - hydroxyethyl) - anilido - 5 - nitroanthraquinone; 1-hydroxy-4-anilido-anthraquinone; 1,8-dihydroxy-4 - m - (alpha - hydroxyethyl) - anilido - 5 - nitroanthraquinone.

45 When an aqueous dyebath is employed, the rate of dyeing may be increased by the use of a suitable dyeing assistant, e.g. pine oil, tripropyl phosphate, tributyl phosphate, diethyl phthalate, methyl salicylate or an N,N-dihydroxyethyl fatty acid amide, such as N,N-dihydroxyethyl capramide. Such dyeing assistants may be applied to the material, as by padding, before dyeing or 50 may be added to the dyebath. As stated, the ethylenically unsaturated O-fading inhibitor may also be applied to the textile material during the dyeing thereof. To this end the inhibitor may be dispersed in the aqueous dyebath if desired.

55 Instead of immersing the textile material in a heated aqueous dyebath the textile material may be colored by applying thereto a printing paste containing the desired dyestuffs. Alternatively the textile material may be colored by passing it through a heated solution of the dyestuff in a liquid polyhydric alcohol such as ethylene glycol. Any other coloring methods known to the art 60 may be employed.

65 As stated, the textile material having a basis of a cellulose ester of low hydroxyl content is given a heat-treatment, preferably during or after the application of the coloring material thereto. This treatment serves to increase the penetration of the dye into the cellulose ester and increases the wash-fastness, resistance to gas-fading, 70 resistance to O-fading and resistance to crocking of the dyed material. Heat-treatment also effects an improvement in the physical properties of the textile material. Thus, it effects an improvement in the safe ironing temperature, its resistance to glazing, its resistance to shrinkage on pressing with moist steam, its resistance to musing or wrinkling on laundering, its resistance to degrada- 75

tion or weakening on exposure to elevated temperatures for long periods of time and its resistance to degradation in sunlight. For example, heat-treatment of a fabric of cellulose acetate of low hydroxyl content raises its safe ironing temperature by at least about 20° C., e.g. up to 220° C. or higher. Heat-treatment generally results in an increase in the crystallinity and crystalline order index of the cellulose ester material.

The conditions of heat-treatment will depend somewhat on the particular textile material being treated, for example, on its weight and construction. In general, when dry heat is used, as when the textile material is passed through a hot air heater, an infra-red heater or in contact with heated rollers or drums, temperatures of 190° C. or above are employed. Preferably, the material is heated to a temperature of about 220 to 235° C. for about 7 to 30 seconds. With lower temperatures, e.g. 190° C., the heating time is considerably longer, for example 5 to 10 minutes. Still lower heat-treatment temperatures may be employed when the heat is applied by means of saturated steam under a pressure of for example 20 to 40 pounds per square inch or by means of a heated bath of ethylene glycol or other polyhydric alcohol. The coloring and heat-treatment may be combined, as by subjecting the textile material for a sufficient period of time to a suitable liquid medium containing a dyestuff dispersed or dissolved therein. For example, the material may be dyed and heat-treated in an aqueous medium maintained under superatmospheric pressure at a temperature of 90° C. or above or in a solution of the dyestuff in hot ethylene glycol. The term "heat-treatment" as employed herein accordingly has reference to high temperature, and the like, as well as treatments at moderate temperatures with solvents or assistants to achieve similar improvements.

If desired, the unsaturated O-fading inhibitors of this invention may be used in combination with amine-type gas-fading inhibitors. In this case the amount and type of amine should be such that there is little discoloration on heat-treating. The polymeric pyridines disclosed in the copending application of Conciatori et al., Ser. No. 488,718, filed February 16, 1955, are very suitable for this purpose and they may be incorporated into the textile material in the same manner as the O-fading inhibitors described above, in the amount of, for example, about 0.5 to 5%, based on the weight of the organic derivative of cellulose textile material. Thus, there may be used 3% of the polymethylvinylpyridine of said copending application and 1% of an unsaturated polyester combined by the reaction of methallyl succinic anhydride and glycol. When the amine-type inhibitor is present discoloration may be reduced by subjecting the textile material to a bleaching agent, after, or preferably before, the heat-treatment operation.

The following examples are given to illustrate this invention further:

#### Example I

A mixture of 1 mole of methallyl succinic anhydride and 1.1 moles of ethylene glycol is heated and stirred under nitrogen atmosphere for 5 hours, on an oil bath kept at 200° C., in a vessel equipped with a condenser for returning vaporized glycol to the mixture. The resulting polyester, which has an acid number of 16 or 17, is purified by dissolving it in a mixture of 90% of methylene chloride and 10% of methanol and boiling the resulting solution in the presence of charcoal.

#### Example II

To a spinning solution containing 21 parts of cellulose acetate of 61.5% acetyl value, in 79 parts of a mixture of 90% of methylene chloride and 10% of methanol there is added 0.63 part of the purified polyester produced in Example I. The solution is spun into yarn and woven into a fabric, which is then dyed with 1-methylamino-4-hydroxy-ethylamino-anthraquinone and there-

after heat-treated by subjecting it to a temperature of 230° C. for 7 seconds in a radiant heat-oven. The fabric is tested for O-fading by the procedure described in the Textile Research Journal, July 1955, volume 25, pages 578 and 579. There is only a very slight change in the color of the fabric, comparison with the original unfaded fabric indicating a shade change rating corresponding to 4 on the International Gray Scale, after 100 hours of the fading exposure. When the above example is repeated, except that the material of Example I is omitted the dyed and heat-treated fabric shows a shade change corresponding to a rating of only 2-3 after 100 hours of fading exposure. In neither case does the heat-treatment, or a subsequent heating for 15 minutes at 200° C., cause any appreciable discoloration of the fabric. Also, both the material containing the unsaturated polyester of Example I and the material containing none of this polyester were equally unaffected by acid dyes under standard wool-dyeing conditions, showing that they could be used for producing cross-dyed effects in wool blends.

When the fabric of this example is tested for O-fading before the heat-treatment it shows no shade change whatever (a rating of 5) after 18 hours of fading exposure and shows a slight change, corresponding to a rating of 3-4 after 100 hours. The corresponding figures for the fabric containing none of the unsaturated polyester of Example I are 3-4 and 1-2 respectively.

#### Example III

A mixture of 1 mole of methallyl succinic anhydride and 1.05 moles of ethylene glycol is heated and stirred under nitrogen atmosphere for 2 hours, on an oil bath kept at 190° C., in a vessel equipped with a reflux condenser for returning vaporized glycol to the mixture and withdrawing water of condensation. The temperature is raised to 210-220° C. for 5 hours longer, the pressure is reduced to 190 mm. Hg and heating is continued for 3 hours. The resulting polyester, which has an acid number of 3.0 and a molecular weight of about 1000, is purified by dissolving it in a mixture of 90% by weight of methylene chloride and 10% by weight of methanol and boiling the resulting solution in the presence of charcoal.

#### Example IV

To a spinning solution containing 21 parts of cellulose acetate of 61.5% acetyl value, in 79 parts of a mixture of 90% of methylene chloride and 10% of methanol there is added 0.63 part of the purified polyester produced in Example III (1 methallyl group unsaturation for 23 anhydroglucoside units) and .01 part of Interchemical Blue B dyestuff, i.e. a mixture of 1,4-bis-methylaminoanthraquinone and 1-methylamino-4-beta-hydroxyethylamino-anthraquinone. The solution is spun into yarn and woven into a fabric, which is then scoured for 10 minutes at 40° C. in a bath containing 1 gram/liter of soap and 1 gram/liter of sodium hexametaphosphate. The scoured fabric is exposed to an O-fading atmosphere for 70 hours and the color is compared with that before exposure. The comparison is made with the Hunter Color Difference Meter which measures the L (grayness), a (redness or greenness) and b (yellow or blueness) of the sample. The number of units of color change  $\Delta E$  is determined according to the following equation:

$$\Delta E = \sqrt{(\Delta L)^2 + (\Delta a)^2 + (\Delta b)^2}$$

The color change is only 5.2 units as compared with 15.3 for a control fabric similarly treated but containing no O-fading inhibitor.

The fabric of this example is about as resistant to gas-fading and ultraviolet light as the control containing no O-fading inhibitor. The presence of the inhibitor does not change the lack of affinity of the yarn for acid dyes under standard wool-dyeing conditions, showing that the 75 inhibitor-containing yarn could be used for producing

7 cross-dyed effects in wool blends. On storage, the viscosity characteristics of the inhibitor-containing dope are the same as those for the dope from which the control fabric is prepared.

*Example V*

(a) Cellulose acetate of 61.5% acetyl value is dissolved to form a 21% by weight solution in a 90-10 weight mixture of methylene chloride-methanol. The solution is divided into a test specimen and a control specimen there being added to the test specimen 3% by weight of the polyester of Example III, based on the cellulose acetate. Both solutions are spun to form filament yarns and the yarns are each woven into fabrics. An inhibitor-containing fabric sample and an inhibitor-free fabric sample are prescoured at 180° F. for one hour in 0.5 gram per liter of soap.

(b) Inhibitor-containing and inhibitor-free scoured and unscoured samples are then dyed with 0.05% by weight of the dyestuff 1,8-dihydroxy-4-p-(beta-hydroxyethyl)-anilido-5-nitroanthraquinone and tested to determine the extent of O-fading after 40 hours' exposure to an O-fading atmosphere. The fabrics containing no inhibitor undergo severe shade changes (a rating of 2) whether or not prescoured. The inhibitor-containing fabric which is not prescoured undergoes a very slight shade change (4-5) while the inhibitor-containing fabric which is prescoured undergoes a slight to moderate change (3-4). This indicates that the inhibitor is resistant to removal by scouring and during dyeing.

(c) Samples of unscoured inhibitor-containing and inhibitor-free fabrics as produced in (a) are dyed for two hours at 176° F. with Eastone Red GLF, i.e. 2-methylsulfone - 4 - nitro - 4' - (N - hydroxyethyl - N - beta-difluoroethyl)-amino-azobenzene. Where the fabric is inhibitor-free its dye content is found to be 0.52% whereas the inhibitor-containing fabric picks up 0.73% of dyestuff, indicating that the inhibitor acts as a dyeing accelerator. The washfastness of the fabrics are equal.

*Example VI*

A mixture of 1 mole of methallyl succinic anhydride and 1.05 moles of ethylene glycol is stirred with an equal weight of xylene under nitrogen atmosphere and heated to reflux using a system to condense and separate water vapor while returning xylene. After the theoretical quantity of water is collected, i.e. in about 4 hours, refluxing is continued for an additional 3 hours. The xylene is then distilled off and the temperature is raised slowly to 200° C. while the pressure is reduced to 5 mm. Hg and held for 20 minutes. After cooling, the polyester is purified as in Example III. Its acid number is 113.0 and its molecular weight is about 1000. It is incorporated into a spinning dope along with dye, spun, and tested as in Example IV. The dyed material after 70 hours exposure to an O-fading atmosphere undergoes a color change  $\Delta E$  of 3.7 units.

*Example VII*

Allyloxypropanediol is substituted for the glycol in Example III to give a product with an acid number of 9.8 and a molecular weight of 850. The ester is incorporated into a spinning dope which is treated as in Example IV. The color change  $\Delta E$  after 70 hours of O-fading is 3.1.

*Example VIII*

The process of Example VII is repeated except that the linear polyester used is the polyester of methallyl succinic anhydride and butene diol, having an acid number of 9.6 and a molecular weight of 700. The color change  $\Delta E$  after 70 hours of O-fading is 4.5 units.

*Example IX*

The linear polyester of maleic anhydride and butene diol, prepared in the same manner as the polyester in

8 Example VI and having an acid number of 5.2 and a molecular weight of 1307, is used in repeating the process of Example IV. The color change  $\Delta E$  is 5.5 units after 70 hours of O-fading.

5

*Example X*

Succinic anhydride and butene diol are substituted for the anhydride and glycol in the process of Example VI and the resulting polyester exhibits an acid number of 1.6 and a molecular weight of 1300. It is used in repeating the process of Example IV and after 70 hours O-fading the fabric undergoes a color change  $\Delta E$  of 5.6 units.

10

*Example XI*

15 A mixed cellulose acetate crotonate having a crotonyl value of 46% and an acetyl value of 20.2% calculated as the combined acids, is prepared as follows:

100 parts by weight of cotton linters are shaken for 2 hours at room temperature with 35 parts of glacial acetic acid. The pretreated linters are cooled to about 10-20° C., and 900 parts of methylene chloride and 400 parts of crotonic anhydride, cooled to 3-5° C., are added. 1 part of perchloric acid is added and the temperature of the mass, which is continuously stirred, starts to increase. A peak temperature of 32-38° C. is reached in 20 minutes, and the vessel which contains the mass is immersed in ice water. Stirring is continued for 40 minutes, at which time the mass becomes a clear amber colored dope. 700 parts of methylene chloride are added, the perchloric acid is neutralized with a slight excess of ammonium hydroxide and the vessel is tumbled for an additional hour. Boiling water is poured into small volumes of the dope causing ebullition of methylene chloride and precipitation of the mixed ester. The mixed ester is washed free of crotonic acid and anhydride with ethanol and then with ether, and is dried first in air and then in an oven at 60° C. for 12 hours. The dried ester is dissolved in a 90/10 weight mixture of methylene chloride/methanol and the solution is combined with a 21 weight percent solution of cellulose triacetate in a 90/10 weight mixture of methylene chloride/methanol. The proportion of cellulose acetate crotonate solution added to the cellulose triacetate spinning dope is varied so that in successive runs the weight percentage of the cellulose acetate crotonate based on the cellulose triacetate is 3%, 4.5% and 10%. The dyestuff employed in Example IV is added to the modified spinning solutions and they are separately spun into filaments, being after treated as in Example IV. The color change  $\Delta E$  after 70 hours of O-fading are respectively 5, 4 and 3 units.

20

25

30

35

40

45

50

*Example XII*

Three parts by weight of cellulose are pretreated for 2 hours with 35% by weight of glacial acetic acid. At 0° C. the cellulose is mixed with an esterification mix comprising 2.5 parts of acetic anhydride, 3.15 parts of acetic acid, 0.82 part of crotonic acid, 0.68 part of crotonic anhydride and 0.21 part of sulfuric acid. A peak temperature of 45° C. is reached in 155 minutes and held for 10 minutes. The resulting dope is mixed with water to precipitate the cellulose mixed ester, which is washed with alcohol, ether and then dried. The ester has a crotonyl content of 4.2% and an acetyl content of 57.7%, calculated as combined acids, and has 0.09 free hydroxyl per anhydroglucose unit. The ester is dissolved, spun into yarn, and woven into a fabric which when subjected to O-fading for 70 hours undergoes a color change  $\Delta E$  of 3.4 units.

55

60

65

70

*Example XIII*

Dopes are prepared as in Example IV, substituting for the inhibitor there disclosed 3% based on the weight of the cellulose triacetate of the following compounds: diethyl phthalate, diallyl phthalate, diallylidene pentae-

rythritol, dicrotonylidene pentaerythritol, triallyl cyanurate, C-oil and the polyester of succinic anhydride and ethylene glycol. Fabrics prepared as in Example IV are tested for color change and the values are given in the following table along with those for fabrics produced in accordance with Examples IV and VI to XII.

|                                                                 | Wt. Percent on Cellulose Triacetate | Units Color Change After 70 Hours O-fading |
|-----------------------------------------------------------------|-------------------------------------|--------------------------------------------|
| None                                                            |                                     | 15.3                                       |
| Diethyl phthalate                                               | 3                                   | 16.0                                       |
| Diallyl phthalate                                               | 3                                   | 4.6                                        |
| Diallylidene pentaerythritol                                    | 3                                   | 5.1                                        |
| Dicrotonylidene pentaerythritol                                 | 3                                   | 4.6                                        |
| Triallyl cyanurate                                              | 3                                   | 4.1                                        |
| C-oil                                                           | 3                                   | 4.6                                        |
| Methallyl succinic anhydride-ethylene glycol, Acid #3           | 3                                   | 5.2                                        |
| Methallyl succinic anhydride-ethylene glycol, Acid #113         | 3                                   | 3.7                                        |
| Methallyl succinic anhydride-propylene glycol, Acid #95         | 3                                   | 3.2                                        |
| Methallyl succinic anhydride butene diol, Acid #9.6             | 3                                   | 4.5                                        |
| Methallyl succinic anhydride-allyloxy-propanediol, Acid #9.8    | 3                                   | 3.1                                        |
| Maleic anhydride-butene diol, Acid #5.2                         | 3                                   | 5.5                                        |
| Succinic anhydride-butene diol, Acid #1.6                       | 3                                   | 5.6                                        |
| Succinic anhydride-ethylene glycol, Acid #18                    | 3                                   | 9.0                                        |
| Cellulose acetate crotonate 46% crotonyl value                  | 3                                   | 5                                          |
| Do                                                              | 4.5                                 | 4                                          |
| Do                                                              | 10                                  | 3                                          |
| Cellulose acetate crotonate yarn, 4% crotonyl value—no additive |                                     | 3.4                                        |

#### Example IV

Three liters of a dyebath containing 1.5 grams of sodium N-methyl-oleyl-taurate, 1.5 grams of sodium hexametaphosphate and 0.09 gram of the dyestuff of Example IV are heated to 95° C. The dyebath is divided into three equal portions, a solution of 0.3 gram of diallyl phthalate in 10 ml. of dioxane being stirred into one portion and a solution of 0.3 gram of triallyl cyanurate in 10 ml. of dioxane being stirred into another portion. Identical 10 gram samples of cellulose triacetate fabric are placed in each of the three dyebaths and removed after 1 hour. The samples are rinsed thoroughly in lukewarm water and dried. Exposure of the fabrics to an oxidizing atmosphere shows that the dyed fabrics treated with the unsaturated additives are much more resistant to color change than the control.

It is to be understood that the foregoing detailed description is given merely by way of illustration and that many variations may be made therein without departing from the spirit of my invention.

Having described my invention, what I desire to secure by Letters Patent is:

1. A heat-treated material exhibiting a safe-ironing temperature of at least 220° C. and having a basis of organic acid esterified cellulose containing at most 0.29 hydroxyl groups per anhydroglucose unit in the cellulose molecule thereof, there being present in said textile material at least one isolated non-conjugated aliphatic carbon-to-carbon unsaturation per 50 anhydroglucose units for protecting said textile material against O-fading when said material is colored with an anthraquinone dye, said unsaturation being present in molecules free of salt-forming groups.

2. A textile material dyed with a dye normally subject to O-fading, said textile material having a basis of organic acid esterified cellulose containing at most 0.29 hydroxyl groups per anhydroglucose unit in the cellulose molecule thereof, there being present in said textile material at least one isolated non-conjugated aliphatic carbon-to-carbon unsaturation per 50 anhydroglucose units for protecting said dye against O-fading, said dye being highly resistant to gas fading as indicated by negligible fading when applied in the amount of 0.3% based on the fabric weight and in the absence of a gas-fading

inhibitor to a textile fabric of cellulose triacetate having an acetyl value of 61.5% by weight calculated as acetic acid and subjected to 3 units of gas-fading exposure in accordance with Test Method 23-52 of the American Association of Textile Chemists and Colorists.

3. A heat-treated textile material exhibiting a safe-ironing temperature of at least 220° C. and having a basis of organic acid esterified cellulose containing at most 0.29 hydroxyl groups per anhydroglucose unit in the cellulose molecule thereof, at least one oxygen atom per 50 anhydroglucose units of the cellulose molecule being bound to a radical containing an isolated non-conjugated aliphatic carbon-to-carbon unsaturation for protecting said textile material against O-fading when said material is colored with an anthraquinone dye.

4. A heat-treated textile material exhibiting a safe ironing temperature of at least 220 °C. and having a basis of cellulose acetate crotonate containing at most 0.29 hydroxyl groups per anhydroglucose unit in the cellulose molecule thereof, there being present at least one crotonyl group per 50 anhydroglucose units for protecting said textile material against O-fading when said material is colored with an anthraquinone dye.

5. A textile material having a basis of an organic acid ester of cellulose and having incorporated therein a minor amount of compatible compound free of basic nitrogen groups and having isolated aliphatic non-conjugated carbon-to-carbon unsaturation for protecting said textile material against O-fading when said material is colored with an anthraquinone dyestuff.

6. A textile material having as basis of a cellulose organic acid ester containing at most 0.29 hydroxy groups per anhydroglucose unit in the cellulose molecule thereof, said cellulose ester having incorporated therein a minor amount of a compatible compound free of salt-forming groups and having isolated non-conjugated aliphatic carbon-to-carbon unsaturation for protecting said textile material against O-fading when said material is colored with an anthraquinone dye, said compound selected from the group consisting of diallyl phthalate, diallyl succinate, acrylic esters of monohydric and polyhydric alcohols, crotonic esters of monohydric and polyhydric alcohols, unsaturated polyesters of polyhydric alcohols and polycarboxylic acids, unsaturated cellulose esters, unsaturated hydrocarbons, unsaturated ethers and unsaturated acetals.

7. A textile material having a basis of cellulose acetate containing at most 0.29 hydroxyl groups per anhydroglucose unit in the cellulose molecule thereof, said cellulose acetate having incorporated therein an unsaturated compound free of basic nitrogen groups and containing a plurality of isolated non-conjugated aliphatic carbon-to-carbon unsaturations.

8. A textile material as set forth in claim 7, in which the unsaturated compound is polymeric and has a molecular weight of at least about 500.

9. A textile material as set forth in claim 8, in which the unsaturations are present in short chains pendant to the main chain of the polymer.

10. A textile material as set forth in claim 7, in which said unsaturated compound is a linear polyester having a molecular weight of at least about 500.

11. A textile material as set forth in claim 7, in which the unsaturated compound is a hydrocarbon polymer.

12. A textile material as set forth in claim 7, in which the unsaturated compound is a cellulose derivative selected from the group consisting of ethers and esters having isolated non-conjugated aliphatic carbon-to-carbon unsaturation, said derivative being present in an amount ranging from about 1 to 10% by weight of the cellulose acetate and including sufficient unsaturations to provide at least one unsaturation for each 50 anhydroglucose units of the cellulose acetate.

13. A textile material as set forth in claim 5, colored with an anthraquinone dye.

14. Process which comprises heat-treating a dyed textile material having a basis of a cellulose organic acid ester containing at most 0.29 hydroxyl groups per anhydroglucose unit in the cellulose molecule thereof, said cellulose ester having incorporated therein an anthraquinone dye and a minor amount of a compatible compound having isolated non-conjugated aliphatic carbon-to-carbon unsaturation free of salt-forming groups and for protecting said dyed material against O-fading.

15. A spinning solution comprising a solution in a solvent comprising methylene chloride, of a cellulose acetate having an acetyl value of at least 61%, calculated as combined acetic acid and, as an inhibitor of O-fading, a minor amount of a compound free of salt-forming groups and having isolated non-conjugated aliphatic carbon-to-carbon unsaturation.

10

15

References Cited in the file of this patent

UNITED STATES PATENTS

|           |                   |               |
|-----------|-------------------|---------------|
| 2,142,007 | Schlack           | Dec. 27, 1938 |
| 2,539,212 | Strobel et al.    | Jan. 23, 1951 |
| 2,702,763 | Pritchard         | Feb. 22, 1955 |
| 2,880,051 | Rosen et al.      | Mar. 31, 1959 |
| 2,892,672 | Conciatori et al. | June 30, 1959 |

OTHER REFERENCES

The Textile Manufacturer, February 1955, pages 71 and 72.

Billmeyer: "Textbook of Polymer Chemistry," Interscience Publisher Inc., N.Y., 1957, page 196.